

Patented June 10, 1924.

1,496,845

# UNITED STATES PATENT OFFICE.

GEORG GRUBE, OF STUTTGART, GERMANY, ASSIGNOR TO METAL & THERMIT CORPORATION, OF CHROME, NEW JERSEY, A CORPORATION OF NEW JERSEY.

## PROCESS OF PRODUCING PURE CHROMIUM BY ELECTROLYSIS.

No Drawing.

Application filed April 13, 1923. Serial No. 631,906.

To all whom it may concern:

Be it known that I, GEORG GRUBE, a citizen of the German Republic, residing at Stuttgart, Germany, have invented certain new and useful Improvements in Processes of Producing Pure Chromium by Electrolysis (for which I have filed an application in Germany on July 19, 1921, and for which further applications have been filed by as-  
signees as follows: Czechoslovakian Republic, September 23, 1922; Switzerland, September 23, 1922; Sweden, September 23, 1922; Austria, September 25, 1922; Norway, September 27, 1922; Great Britain, September 28, 1922; Belgium, October 17, 1922; Italy, October 24, 1922; and France, October 30, 1922), of which the following is a specification.

Pure chromium, free of carbon, has been manufactured heretofore principally by aluminothermical means or in the electric furnace. Attempts have been made to produce chromium metal by electrolysis, but it has not been possible to produce thick precipitates of uniform density in a reliable manner by means of the processes heretofore employed. The precipitates formed by such processes have scaled off after reaching a certain thickness or have been deficient in uniformity or otherwise unfit for use.

The present invention relates to an electrolytic process by means of which not only thin but also thick deposits of pure chromium may be produced in a continuous manner, said process involving the use of an electrolytic bath containing as initial ingredients chromium trioxide ( $Cr_2O_3$ ), chromic hydroxid ( $Cr(OH)_3$ ), and an acid other than chromic acid capable of dissolving chromic hydroxid, the amount of chromium trioxide being equal to at least twice the amount of the chromic hydroxid and the acid together. In order to obtain satisfactory results the chromic hydroxid content of the bath should be in excess of the quantity necessary to neutralize the acid content of the bath.

The deposition of the chromium may be effected upon any kind of metallic parts, such for example upon iron or copper or upon nickel coated iron. As an anode lead-hyperoxid is preferably employed, the relative sizes of the anode and cathode being so proportioned that all lower oxides of chro-

mium produced at the cathode and not reduced to metal nor being obtained in metallic condition, are subjected to a higher degree of oxidation at the anode with formation of chromium-trioxide.

The process may for instance be carried out in the following manner: Into an electrolytic decomposition vessel filled with water a sufficiency of chromium-trioxide, sulphuric acid and chromic hydroxid are introduced that in each liter of the solution there are contained 250 g.  $CrO_3$ , 3 g.  $Cr_2(SO_4)_3$  and 6 g.  $Cr(OH)_3$ . Such a solution is obtained by using for each liter of water 250 g.  $CrO_3$ , 2.25 g.  $H_2SO_4$  and 7.58 g.  $Cr(OH)_3$ . The solution is submitted to electrolysis at the temperature of the room without the use of a diaphragm and at a current density of 10 amp. per square decimeter at the cathode, and a current density of 5 amp. per square decimeter at the anode. Thus for instance a current of 3.2 to 3.4 volts and 30 amp. current strength was employed with two lead-hyperoxid anodes of about 3 square decimeter each active surface and in parallel connection between which the cathode of 3 square decimeter surface consisting of copper sheet was suspended. During the procedure  $CrO_3$  in solid condition was added in such a manner that the contents of the electrolyte of  $Cr_2(SO_4)_3$  and  $Cr(OH)_3$  remained unchanged and that only the chromic acid was reduced to metallic chromium. Under the conditions mentioned in 100 hours 300 g. pure chromium were precipitated for which purpose 577 g.  $CrO_3$  had to be introduced into the solution.

The operation could be carried on for months continuously and yielded layers of chromium of any desired thickness; it was even possible to obtain the precipitated chromium in a highly glossy condition.

The chromium adheres with considerable tenacity to a chromium-coated piece of sheet iron, so that said sheet iron could be frequently bent and worked without the least liability of the chromium to become detached. It is a particular advantage of the process that it is possible to produce highly brilliant chromium precipitates upon a polished carrier of some other metal such as iron, copper or brass, so that the objects which have been coated with chromium in this manner may be directly employed with-

out any subsequent polishing. It is evident moreover, that other metals may be precipitated upon the metallic chromium thus produced by electrolysis, so that such metals 5 will firmly adhere thereto. On the other hand, the surface of a cathode may be prepared by well known means, by very slight greasing for instance, so that a layer of chromium precipitated thereon may be 10 readily detached.

By the subsequent heating of chromium coated metals preferably in an indifferent or inert gas the different metals may be alloyed with each other completely or to any 15 desired extent.

It should be pointed out that my invention is not restricted to the particular proportions, current densities and conditions hereintofore referred to, but that such conditions and percentages may vary to suit existing conditions and other changes and modifications may be made in accordance with local requirements and the convenience of the operator, and without deviating from 25 the spirit of my invention as pointed out in the claims.

What I claim is:

1. Process of producing pure metallic chromium which consists in electrolyzing a 30 solution formed by mixing water, chromium trioxid, chromic hydroxid and an acid other than chromic acid capable of forming a soluble chromium salt by reaction with chromic hydroxid, the chromium trioxid 35 being equal to at least twice the total amount of the chromic hydroxid and acid.

2. Process of producing pure metallic chromium which consists in electrolyzing a 40 solution formed by mixing water, chromium trioxid, chromic hydroxid, and an acid other than chromic acid capable of forming a soluble chromium salt by reaction with chromic hydroxid, the chromium trioxid being equal to at least twice the total 45 amount of the chromic hydroxid and acid, and the chromic hydroxid being in excess of the quantity necessary for the neutralization of the acid.

3. Process of producing pure metallic 50 chromium which consists in electrolyzing an aqueous bath containing chromium trioxid, chromic hydroxid and a soluble chromium salt, the total amount of the chromic hydroxid and chromium salt being less than 55 half of the amount of the chromium trioxid in the bath.

4. Process of producing pure metallic chromium which consists in electrolyzing an

aqueous bath containing chromium trioxid, chromic hydroxid and a soluble chromium salt, the chromium trioxid being equal to 60 at least twice the amount of the chromic hydroxid and chromium salt, and regulating the current densities at the electrodes so as to produce anodic oxidation into chromic compounds of the chromium compounds of 65 a lower state of oxidation formed at the cathode.

5. The process of producing pure metallic chromium which consists in electrolyzing an 70 aqueous bath, containing chromium trioxid, chromic hydroxid and chromic sulphate the total amount of the chromic hydroxid and of the chromic sulphate being less than half the amount of the chromium trioxid present.

6. Process of producing pure metallic chromium which consists in electrolyzing an aqueous bath containing chromium trioxid, chromic hydroxid and a soluble chromium salt, the chromium trioxid being equal to 75 80 at least twice the amount of the chromic hydroxid and chromium salt, and regulating the current densities at the electrodes so as to produce anodic oxidation into chromium trioxid of the lower oxides of 85 chromium formed at the cathode.

7. Process of producing pure metallic chromium which consists in electrolyzing an aqueous bath containing chromium trioxid, chromic hydroxid and a soluble chromium 90 salt, the chromium trioxid being equal to 95 at least twice the amount of the chromic hydroxid and chromium salt, and regulating the current densities to approximately ten amperes per square decimeter at the cathode and approximately five amperes per square decimeter at the anode.

8. Process of producing pure metallic chromium which consists in electrolyzing an aqueous bath containing chromium trioxid, chromic hydroxid and a soluble chromium salt, the chromium trioxid being equal to at least twice the total amount 100 of the chromic hydroxid and the chromium salt, adding chromium trioxid to the solution during the electrolysis at a rate corresponding to the rate of deposition of metallic chromium, and correspondingly regulating the relative current densities at the electrodes, thereby maintaining the composition 105 of the bath substantially unchanged during the electrolysis.

In testimony whereof, I affix my signature.

GEORG GRUBE.